

1

2,758,085

**METHOD FOR INCORPORATING OIL-INSOLUBLE, SOLID ADDITION AGENTS IN MINERAL OILS**

Edward A. Oberright, Woodbury, N. J., assignor to Socony Mobil Oil Company, Inc., a corporation of New York

No. Drawing. Application June 8, 1953,  
Serial No. 360,349

4 Claims. (Cl. 252—25)

This invention relates generally to improved lubricating oil compositions. More particularly, it relates to a novel means for the incorporation of certain improving agents into lubricating oils and to a novel form of such addition agents.

As is well known, it is the practice in the art today to add to lubricating oils minor amounts of chemical agents to improve various lubricating characteristics of such oils. A great number and variety of such improving agents are known. The present invention is directed primarily to solid lubricating oil addition agents of the inorganic type which are insoluble in lubricating oils. These include particularly the oxides, hydroxides and carbonates of the alkali and alkaline earth metals, such as potassium hydroxide, sodium hydroxide, calcium oxide, calcium hydroxide, calcium carbonate, barium hydroxide, strontium hydroxide, zinc oxide, etc. However, the principle of the invention is applicable to solid inorganic type, oil-insoluble addition agents in general. Although these additives are insoluble in engine lubricating oils, they may be dispersed therein and, when so dispersed, they provide highly desirable improvements in the oil. Thus, they inhibit increase of acidity of the oil in use so that corrosion of the engine parts with which the oil comes in contact is substantially reduced. They also improve the detergent character of the oil, so that the deposition of sludge on the engine parts is effectively reduced. Due to the high effectiveness thus exhibited by these additives, as well as their relatively low cost and availability, their use in engine oils is highly desirable. However, the fact that they are insoluble in the oil constitutes a serious drawback to their use from the marketing angle. Thus, the oil containing the dispersed additive has a cloudy appearance. Also, on long standing the additive tends to settle out of the oil. Actually, the cloudy appearance of the oil does not detract from its quality, nor does the settling out of the additive affect its efficiency since, in the engine, the additive is redispersed in the oil whenever the engine is started up. However, the cloudy appearance of the oil creates a doubt in the customers' mind as to its quality. A way of utilizing the inorganic addition agents which would solve the problem of customer resistance was, therefore, sought. A possible solution which suggested itself was that these additives could be marketed separately for addition to the oil at the point of use, i. e., in the engine, rather than at the point of manufacture. In this way, the beneficial use of these additives would be attained while the marketing problem would be eliminated. Such a manner of use, however, posed the further problem of supplying the additives in a form which would be convenient for handling and which at the same time would be efficiently dispersible in the oil. To give a ready dispersion in the oil, these solid, inorganic additives must be added to the oil in finely divided form; i. e., the particle size should be no greater than about 45 microns. Distribution of the additives in this form, however, would not be feasible for several reasons. In the first place, it would be costly, since separate, weighed portions, or dosages, of the additives would have

2

to be prepared and packaged in some manner for such distribution. Also, this form of the additive would be unattractive from the marketing angle. The object of this invention is, therefore, to provide a means for the utilization of these additives which is convenient and practicable as well as attractive from the marketing standpoint. A further object is the provision of a novel form of these addition agents for addition to lubricating oils at the point of use. Other and further objects of the invention will become apparent from the following description thereof.

The present invention provides a most convenient and practicable form of the solid, inorganic, oil-insoluble addition agents. This novel form of additive comprises solid, composite pellets of the finely divided additive and a wax binding material. In this form the additives may be added to the lubricating oil at the point of use, such as in the crankcase of an engine, and provide a ready dispersion of the additive in the oil.

In accordance with the invention, the additive is prepared as follows: The additive is ground, if necessary, and passed through a 325-mesh screen to provide a particle size not greater than approximately 45 microns. A wax, such as a paraffin wax, is heated above its melting point and the comminuted additive is mixed with the liquid wax, with stirring, to provide a homogeneous dispersion of the additive in the wax. This mixture is then formed into pellets in any suitable manner, such as by pouring it into molds and allowing it to cool and solidify.

The unique advantage of the pellets of the invention is that the additive is maintained therein in a finely divided, readily dispersible, state. Upon addition of the pellets to the oil, the wax component dissolves and the finely divided additive is simultaneously dispersed in the oil. Compacted pellets of the addition agents per se, on the other hand, will not give a satisfactory dispersion of the additive in the oil, even when the engine is operated for a considerable period.

The wax used in forming the pellets of the invention may be any oil-soluble wax, or wax-like material, which is solid at temperatures up to at least 100–125° F. Suitable waxes are, for example, paraffin wax, japan wax, carnauba wax, beeswax, spermaceti, 1-octadecanol, etc., paraffin wax being particularly preferred.

The following examples show the utility of the invention from the standpoint of providing the effective dispersion of solid addition agent upon addition to the lubricating oil in an internal combustion engine.

## EXAMPLE I

### Zinc oxide-wax pellets

Zinc oxide was prepared in the form of zinc oxide-wax pellets as follows. Powdered zinc oxide was passed through a 325-mesh screen to provide a particle size of not greater than 45 microns and then mixed with hot, liquid paraffin wax (melting point 120–125° F.) and the heated mixture stirred thoroughly. The mixture was then poured into a series of molds and allowed to cool and solidify. The pellets thus obtained contained 40% by weight of zinc oxide.

The pellets were tested in the Lauson Oxidation Stability Test OS-2. This test involves the operation of the single cylinder, 4-cycle, liquid cooled engine for 100 hours under the following conditions:

|                          |   |               |
|--------------------------|---|---------------|
| Oil temperature          | — | °F. 270       |
| Jacket temperature       | — | °F. 212       |
| Speed                    | — | R. P. M. 1825 |
| One-half throttle        | — |               |
| 13.0-1 air-fuel ratio    | — |               |
| Oil added every 20 hours | — |               |

The test determines oil deterioration as primarily indi-

cated by corrosion of the copper-lead bearing and secondarily by engine cleanliness. The copper-lead bearing of the engine is accurately weighed before and after the test run and the loss in weight thereof recorded. The engine which is clean at the start of the test is inspected after the test run for cleanliness of the rings, lands, ring grooves and piston skirt. Cleanliness ratings are made, based on a scale of from 100 to zero, a rating of 100 signifying a perfectly clean engine and a rating of zero representing the worst possible deposit condition.

To test the pellets, a sufficient number thereof were added to the base oil, an S. A. E. 20 grade Pennsylvania motor oil, in the crankcase of the engine, via the oil addition tube, to give a 0.5% weight concentration of zinc oxide in the oil. With each addition of make-up oil, sufficient pellets were added to maintain this original additive concentration. The fuel used was a blended gasoline comprising 40% thermal plus 30% catalytically cracked plus 30% straight run plus 2.5 cc. of TEL. A control test was also conducted on the base oil alone.

The test with the base oil alone showed a bearing weight loss of 394 milligrams per half-bearing and an engine cleanliness rating of 77, while the test utilizing the zinc oxide-wax pellets showed a bearing weight loss of 76 milligrams per one-half bearing and an engine 25 cleanliness rating of 82.

#### EXAMPLE II

##### Calcium hydroxide-wax pellets

A high grade of calcium hydroxide, known as Grease-maker's Lime, was ground and passed through a 325-mesh screen and stirred into hot, liquid scale wax (melting point 125-127° F.). The stirring was continued for ½ hour after the addition of the lime to insure a homogeneous mixture. The mixture was then poured into molds and allowed to cool and solidify. The pellets thus obtained contained 31% by weight of calcium hydroxide.

The pellets were tested in the Lauson D-4A Detergency Test. This test involves the operation of the single cylinder, 4-cycle, liquid cooled engine for 100 hours under the following conditions:

|                          |          |      |
|--------------------------|----------|------|
| Oil temperature          | °F.      | 225  |
| Jacket temperature       | °F.      | 275  |
| Speed                    | R. P. M. | 1825 |
| Brake load               | H. P.    | 1.6  |
| One-half throttle        |          |      |
| 13-1 air-fuel ratio      |          |      |
| Oil added every 20 hours |          |      |

This test determines the effectiveness of the lubricating oil in preventing fouling as measured by the cleanliness of the rings, lands, ring grooves and piston skirts. Engine cleanliness ratings are assigned on a scale of 100 to zero in the same manner as for the Lauson OS-2 Test.

To test the calcium hydroxide-wax pellets, a sufficient number of the pellets were added to the base oil in the crankcase of the engine, via the oil-addition tube, to provide 1% by weight of calcium hydroxide in the engine oil. The base oil used was an S. A. E. 20 grade Pennsylvania motor oil. With each addition of make-up oil during the test run, sufficient pellets were added to maintain this original additive concentration. The fuel used was the same as defined in Example I. A test was conducted on the base oil also as a control.

The test conducted on the oil alone gave an engine cleanliness rating of 65, while the test using the calcium hydroxide-wax pellets gave a rating of 80.

The size of the pellets and the proportion of additive therein can, of course, be controlled. The pellets may contain as little as about 10% and up to 90% of the additive. Generally, it is preferred to so design the pellets that one pellet will supply the required improving amount of additive for a specified quantity of oil. The

number of pellets to be added in any case is then determined by the volume of oil to be treated. For use in automobile engines the pellets will be of relatively small size since the amount of additive required is ordinarily small, i. e., from about 0.1% to about 10% by weight; and, a pellet comprised, for example, of 50% addition agent and 50% binding material and weighing 16 grams will supply 1% of additive to one quart of oil.

Although, as heretofore indicated, the principle of this invention is primarily applicable to the incorporation in oil of the solid, oil-insoluble, inorganic-type addition agents, it will be appreciated that it may be advantageously applied to any solid-type additive, including the elemental metals and solid, oil-soluble, organic addition agents, since it provides a convenient means of adding controlled amounts of such additives to the oil at the point of use, whereby the oil is fortified to meet special operational conditions, or refortified as the addition agents originally present therein become depleted by use. 20 The invention may also find useful application in the addition of additives to hydrocarbon fractions, other than lubricating oils, such as fuel oils, gasolines, etc.

Having now fully described the invention, what is claimed as new and patentable is:

1. A method for incorporating an oil-insoluble, solid, addition agent into a mineral oil fraction, which comprises (1) comminuting the addition agent to an average particle size no greater than about 45 microns, (2) forming a compacted pellet comprising from about 10% to about 90%, by weight, of the comminuted addition agent and from about 90% to about 10%, by weight, of a wax binder and (3) adding the said pellet to the mineral oil fraction.

35 2. A method for incorporating a solid, inorganic basic compound, selected from the group consisting of the metal oxides and hydroxides of the metals of Group II of Mendeleeff's Periodic Table of the Elements, into a mineral lubricating oil which comprises (1) comminuting the said compound to an average particle size no greater than about 45 microns, (2) forming a compacted pellet comprising from about 10% to about 90%, by weight, of the comminuted solid basic compound and from about 90% to about 10%, by weight, of a wax binder and (3) adding the said pellet to the oil.

30 3. A method for incorporating solid zinc oxide into a mineral lubricating oil which comprises (1) comminuting the zinc oxide to an average particle size no greater than about 45 microns, (2) forming a compacted pellet comprising from about 10% to about 90%, by weight, of the comminuted zinc oxide and from about 90% to about 10%, by weight, of a wax binder and (3) adding the said pellet to the oil.

35 4. A method for incorporating solid calcium hydroxide into a mineral lubricating oil which comprises (1) comminuting the calcium hydroxide to an average particle size no greater than about 45 microns, (2) forming a compacted pellet comprising from about 10% to about 90%, by weight, of the comminuted calcium hydroxide and from about 90% to about 10%, by weight, of a wax binder and (3) adding the said pellet to the oil.

#### References Cited in the file of this patent

##### UNITED STATES PATENTS

|    |           |                  |       |               |
|----|-----------|------------------|-------|---------------|
| 65 | 1,699,274 | Bohart           | ----- | Jan. 15, 1928 |
|    | 2,079,051 | Sullivan         | ----- | May 4, 1937   |
|    | 2,110,503 | Duckham          | ----- | Mar. 8, 1938  |
|    | 2,292,047 | Calhoun          | ----- | Aug. 4, 1942  |
|    | 2,485,861 | Campbell et al.  | ----- | Oct. 25, 1949 |
| 70 | 2,671,758 | Vinograd et al.  | ----- | Mar. 9, 1954  |
|    | 2,676,925 | Lindstrom et al. | ----- | Apr. 27, 1954 |

##### FOREIGN PATENTS

|         |               |       |              |
|---------|---------------|-------|--------------|
| 360,121 | Great Britain | ----- | Nov. 5, 1931 |
|---------|---------------|-------|--------------|